

J. F. MONNOT.  
COMPOUND METAL OBJECT.  
APPLICATION FILED JULY 16, 1908.

960,372.

Patented June 7, 1910.

Fig. 1.



Fig. 2.



Fig. 4.



Fig. 3.



Attest:

Emmett  
Frank E. Hoffmann

by

Inventor:  
J. F. Monnot  
Marblehead, Mass.  
Atty

# UNITED STATES PATENT OFFICE.

JOHN F. MONNOT, OF NEW YORK, N. Y., ASSIGNOR TO DUPLEX METALS COMPANY, OF NEW YORK, N. Y., A CORPORATION OF NEW YORK.

## COMPOUND-METAL OBJECT.

960,372.

Specification of Letters Patent. Patented June 7, 1910.

Application filed July 16, 1908. Serial No. 443,796.

*To all whom it may concern:*

Be it known that I, JOHN F. MONNOT, a citizen of the United States, residing at New York, in the county of New York and State of New York, have invented certain new and useful Compound-Metal Objects; and I do hereby declare the following to be a full, clear, and exact description of the same, such as will enable others skilled in the art to which it appertains to make and use the same.

My invention relates to compound metal objects comprising objects having an inner or body portion composed of soft and ductile metal, such as copper, and a weld-united outer portion of harder and stronger metal, such as steel. Electrical conductor wire comprising a core of high-conductivity metal, such as copper, and a shell of harder or stronger metal, such as steel, is desirable for many purposes, as its electrical properties are in many respects different from ordinary copper wire, or from steel-cored copper-coated wire, even though the copper-coating of such wire be quite thick. The steel coated copper wire gives to a circuit quite a different "loading" from that given by an ordinary copper wire, or a steel-cored copper wire of equivalent ohmic resistance, thus often making unnecessary the inclusion of special inductive resistance in the circuit, or greatly reducing the special inductive resistance required, and distributing the inductance of the circuit more uniformly over the line than can be done by the inclusion at intervals of inductive resistance. A steel-clad copper wire having coating and core weld-united at all points between abutting surfaces, and, therefore, in uniform electrical union at all such points, has different properties electrically from a similar wire in which the two metals are only in mechanical contact and in which, therefore, the electrical connection between the two metals is less perfect and uniform, not all points between abutting surfaces being in equally good electrical union, allowing the possibility of local circuits. Where, as is usually the case, there are spots of oxid between the two metals, this is still more likely to take place. The steel coated copper wire is also stiffer than the steel-cored copper wire, for corresponding amounts of metal, the stronger and stiffer steel being in the mechanically

stronger tubular form, and this greater 55 stiffness is, under some conditions, desirable.

The steel coated wire may have its outer surface protected by a thin layer of copper or other suitable material which will serve to prevent oxidation or like chemical attack of 60 the steel surface. Such a thin outer coating will not materially affect the electrical properties of the conductor desired for the present purposes.

Steel coated material such as described 65 may be made most readily by forming an ingot comprising a steel coating and a core of copper or other metal of high conductivity, with or without an outer coating to protect the outer surface of the steel, ac- 70 cording to the method described in my companion application of even date herewith, Ser. No. 443,797, (Patent No. 927,062, dated July 6, 1909) and then extending this ingot by the usual methods of working to produce 75 wire or the like of the desired size. Such method of forming ingots is illustrated in Figure 1 of the accompanying drawings, in which drawings:

Fig. 1 shows a central vertical section of a 80 mold, pouring funnel, and an ingot therein formed as herein described; Figs. 2, 3 and 4 show sections of different conductors embodying my present invention.

Referring first to Fig. 1, 1 designates a 85 circular two-part mold provided with cooling means 2, which in the instance shown is a hollow jacket through which cooling water, oil, etc., are circulated; or compressed air or other suitable gas may be expanded 90 in the jacket space for the purpose of absorbing heat. In the construction shown the mold is assumed to be of metal, iron molds being permissible in casting copper and like metals inside a steel shell or be- 95 tween a steel shell and the sides of the mold, according to the method referred to. But in lieu of a metal mold, a mold of refractory material, for example, a mold of homogenized carbon, such as illustrated and de- 100 scribed in my application Ser. No. 430,097, (Patent No. 928,470, dated July 20, 1909) may be used. Suitable means as for example bands 3 and wedges 4, as shown, are provided to prevent separation of the sections of the mold during the casting, and until the cast metal has solidified. A sec- 105 tional mold is employed instead of the one

piece mold commonly used in casting ingots simply because it is desirable in many cases that the ingot produced shall have no draft vertically; otherwise a one piece mold would be used.

5 designates a shell or tube of steel or iron to form the steel coating of the resulting article, its thickness being properly proportioned, with reference to the diameter of the ingot, so that this steel shell when extended or drawn down to final size to form a finished article will have the desired thickness. This steel shell, before it is placed in the ingot mold, may have been thinly coated 10 by dipping it for a brief interval in supermolten copper or other suitable supermolten coating metal, according to the method set forth in my Patent No. 853,716, in which patent I have set forth a method of producing clad metals based upon the fact that while copper and like metals do not form any weld-union when contacted at ordinary casting temperatures with a clean steel surface, yet such a weld union is formed when 15 the copper or like metal with which the steel is contacted is heated to a considerably higher temperature, termed by me in said patent, for the sake of a name, the "supermolten temperature". And as set forth in 20 said patent, a steel object immersed momentarily in a bath of such supermolten unlike metal and then withdrawn under conditions precluding oxidation, will be found covered with a thin welded-on coating of metal of 25 the supermolten bath, and with this coating copper and many other metals when cast thereagainst at ordinary casting temperatures or slightly higher temperatures, will unite readily and inseparably. Or, the steel 30 shell may have had its surface treated with a vapor of zinc or like metal as set forth in the application of W. M. Page, Ser. No. 443,339, filed July 13, 1908, (Patent No. 949,837, dated February 22, 1910) so pro- 35 ducing a surface with which molten copper and like metals at ordinary casting temperatures will unite readily and inseparably; or, the said steel shell may have been 40 heated to a very high white heat before it 45 is placed in the mold so that the molten metal cast within or within and around said shell will be raised, in the immediate vicinity of said shell, to the supermolten condition. Or, as an alternative to the above 50 methods, the copper or like metal may be cast within, or within and around, such shell, while in the supermolten condition.

55 6 designates a suitable pouring tile or funnel, which may be of refractory material, such as fire clay, or carbon, or may be of metal. In the particular instance shown the shell 5 is of somewhat smaller diameter than the interior diameter of the mold, in order that molten metal may be cast without 60 as well as within said shell and therefore the

pouring tile 6 is provided not only with a central space 7 for the introduction of the molten metal for the core, but also with side spaces 8 for the introduction between the shell 5 and the mold of molten coating 70 metal.

The metal cast within or within and around the shell 5, is preferably cast through a deep layer of molten wiping material 9, according to the methods set forth 75 in my application Sr. No. 391,674 (Patent No. 929,688, dated August 3, 1909) and my application Serial No. 443,298 (Patent No. 929,687, dated August 3, 1909). Such molten wiping material removes oxid impurities and occluded and entrained gases and insures a particularly dense, tough and homogeneous casting, free from blow holes, blebs, etc.; also if this wiping material contains a considerable proportion of oxid-dis- 80 solving ingredient the mold need be only partly filled with this wiping material prior to the introduction of the molten metal, the molten metal flowing down through this wiping material as it is cast and so displacing upward the wiping material, which is of less specific gravity, said wiping material as it rises progressively freeing the surface of the shell 5 and, when metal is cast between said shell and the sides of the mold, 85 also freeing the mold walls, of oxid or like impurities, absorbed gases, etc. A suitable wiping material is borax or a mixture of borax and sodium or potassium silicate to which a little fluor spar may be added. The 90 proportions of the ingredients of the wiping material may be varied as required to produce a material which will be freely liquid at the temperature at which the molten metal is cast. This wiping material may, 95 if desired, be placed in the mold solid, since the first of the molten metal introduced into the mold will melt it; or if the shell 5 be placed at a white heat in the mold, the heat from this shell will suffice in general to melt 100 solid wiping material placed within the mold.

The shell 5 and the wiping material having been placed in the mold as specified, molten copper or other metal to form the 105 core and, if an outer coating is desired, to from this shell will suffice in general to melt mold and in passing through the molten wiping material is cleansed as above described, and caused to contact with the surface of the shell 5, and is permitted to solidify against such surface, thereby welding to said surface. Commonly the molten metal will be cast in such quantities as not only to 110 completely fill the mold but also to rise somewhat into the passage or passages of the pouring funnel 6, and owing to the covering of molten wiping material, which material is of low heat conductive capacity, 115 and to the refractory nature of funnel 6 120

125 130

when said funnel is of carbon, clay etc., the head of molten metal within this funnel will be relatively slow to solidify, and so will fill in any spaces left by contraction of the metal below, the hydrostatic pressure due to this additional height of molten metal and of the wiping material above it further tending to insure a tough dense cast metal free from blow holes and the like.

10 If desired, the molten metal cast between the shell 5 and the walls of the mold, may be cast after the casting of the metal within said shell, and after such metal within the shell has begun to solidify, the shrinkage of 15 the metal cast outside of the shell so tending to force the contraction of the shell to keep pace with the contraction of the metal cast within it, and such contraction may be hastened by the circulation of cooling fluid 20 through the jacket 2, the rapid cooling so produced also improving the quality of the cast metal, if it be copper or like metal, and preventing any attack of the metal of the mold, if the mold be of metal, by the cast 25 metal, if the latter be cast at supermolten temperature; and this rapid cooling further tends to prevent attack of the metal of the shell by the cast metal, if the latter be cast at supermolten temperature, to such extent 30 as to contaminate the cast metal.

The ingot so produced may be worked in the ordinary manner, either immediately after solidification, or after submission to a soaking heating, and may be rolled and 35 drawn down to final size and shape in the ordinary manner.

In co-extending the joined metals the softer core metal being compressed inside the steel shell while prevented from lateral 40 yielding or extrusion by its weld-union to such steel, assumes a peculiar hard texture, analogous to the surface texture of hard drawn wire, increasing its strength materially.

45 In Fig. 2 I have shown in enlarged section, a wire so produced, comprising a core 10 of copper or like metal of high conductivity, a coating 11 of steel and an outer coating 12 of copper or like material. This 50 outer coating may be of any thickness desired. It may be very much thinner relatively, than as shown in Fig. 2, or it may be very much thicker, as shown in Fig. 3. It 55 is not necessarily the same metal as that of the core 10. In most cases the principal function of this outer coating 12 will be to protect the steel coating 11 from oxidation or like chemical attack; therefore it may be very thin. But in many cases the outer coating 60 12 of non-ferrous metal may be omitted altogether, and in Fig. 4 I have shown such a wire.

The metal may of course be rolled or worked to various shapes other than the circular shape illustrated, and I do not limit

myself to any particular shape of the final product.

What I claim is:—

1. A clad metal article comprising a non-ferrous core and an enveloping tubular ferrous metal coating weld-united to each other and in electrical union at all points of abutting surfaces. 70

2. A clad metal article comprising a core of cupriferous metal and an enveloping tubular coating of ferrous metal weld-united to each other and in electrical union at all points of abutting surfaces. 75

3. A clad metal article comprising a copper core and an enveloping tubular ferrous metal coating weld-united to each other and in electrical union at all points of abutting surfaces. 80

4. A clad metal article comprising a non-ferrous core and a ferrous metal coating weld-united to each other, and another coating of non-ferrous metal surrounding said ferrous coating. 85

5. A clad metal article comprising a core of cupriferous metal and a coating of ferrous metal weld-united to each other, and another coating of non-ferrous metal surrounding said ferrous coating. 90

6. A clad metal article comprising a copper core and a ferrous metal coating weld-united to each other, and another coating of non-ferrous metal surrounding said ferrous coating. 95

7. A clad metal article comprising a non-ferrous core and a ferrous metal coating weld-united to each other and another coating of cupriferous metal surrounding said ferrous coating. 100

8. A clad metal article comprising a core of cupriferous metal and a coating of ferrous metal weld-united to each other and another coating of cupriferous metal surrounding said ferrous coating. 105

9. A clad metal article comprising a copper core and a ferrous metal coating weld-united to each other, and another coating of cupriferous metal surrounding said ferrous coating. 110

10. A clad metal article comprising a non-ferrous core and a ferrous metal coating weld-united to each other and another coating of copper surrounding said ferrous metal. 115

11. A clad metal article comprising a core of cupriferous metal and a coating of ferrous metal weld-united to each other and another coating of copper surrounding said ferrous metal. 120

12. A clad metal article comprising a copper core and a ferrous metal coating weld-united to each other, and another coating of copper surrounding said ferrous metal. 125

13. An extended metal article comprising a core of non-ferrous metal and a tubular coating of ferrous metal weld-united and 130

co-extended said joined metals being electrically united at all points of abutting surfaces.

14. An extended metal article comprising  
5 a core of cupriferous metal and a tubular coating of ferrous metal weld-united and co-extended said joined metals being electrically united at all points of abutting surfaces.

- 10 15. An extended metal article comprising

a core of copper and a tubular coating of ferrous metal weld-united and co-extended said joined metals being electrically united at all points of abutting surfaces.

In testimony whereof I affix my signature, in the presence of two witnesses.

JOHN F. MONNOT.

Witnesses:

H. M. MARBLE,  
FRANK E. RAFFMAN.